

# UNITED STATES PATENT OFFICE.

WILLIAM WEIMAR, OF APPLETON, WISCONSIN.

## METHOD OF TREATING FIBROUS MATERIALS.

1,375,125.

Specification of Letters Patent. Patented Apr. 19, 1921.

No Drawing.

Application filed February 5, 1920. Serial No. 356,534.

To all whom it may concern:

Be it known that I, WILLIAM WEIMAR, a citizen of the United States, residing at Appleton, in the county of Outagamie and State of Wisconsin, have invented certain new and useful Improvements in Methods of Treating Fibrous Materials, of which the following is a specification.

This invention relates to processes for treatment of fibrous material, such as wood or the like.

One of the objects of the invention is to provide an improved process for the treatment of wood, wood pulp or fiber, fiber board, card board and other similar substances or material whereby to render them water proof, weather proof, and substantially immune from the effect of dry rot, vegetable fungoid and microbic organisms.

Another object is to change the color of the treated wood, to a dark brown or black, to enhance its appearance and to improve its texture.

Another object is to remove any objectionable odors from the treated material.

Another object is to render the treated wood, or similar fibrous material more plastic, or less brittle, and to fill the pores so that it will take on a higher finish or polish.

Other, further and more specific objects of the invention will become readily apparent, to persons skilled in the art, from a consideration of the following description.

The object sought in carrying the invention into effect is to drive out of the pores of the wood any resident content and then to coat the pores with a liquid preservative and finally to fill them with the preserving and insulating compound. The mode of procedure is substantially as follows:—

The bodies of wood, or pieces of suitable sizes, are first immersed in a twenty per cent. solution of sodium carbonate. The solution is maintained hot and the wood should remain in the solution, preferably, twenty-four hours, or until the solution has thoroughly impregnated the wood body. The wood may first have been kiln dried or green wood may be used if the preserving solution is heated sufficiently above the boiling point. This will drive out the sap and allow the entrance of the solution into the pores. From this solution the wood is removed and allowed to dry, or is dried superficially.

The wood after being treated with the sodium carbonate and dried is then immersed in hot hydro-carbon liquid, until the pores are well coated, after which it is taken from the hydro-carbon and allowed to dry until it is no longer "sticky". It is then placed in a vat or other suitable receptacle containing hot or molten sulfur and resin. I have found that sufficient sulfur should be used to submerge the wood and that very good results may be obtained from the resin of commerce, about one per cent. in weight, of the sulfur, or ninety per cent. of sulfur and one per cent. of resin may be satisfactorily used.

The fibrous material should be maintained in this last mentioned heated solution until it assumes the desired color and weight. The time required for this treatment depends, to some extent, upon the character of the body of material operated upon. For example, in the treatment of close grain wood, the time that it shall remain in the heated sulfur and resin solution, varies from three to seven days.

After the substance has been cooked in the sulfur solution, for the requisite period of time, it is then taken out and rapidly cooled. This may conveniently be done by immersing it in cold water or by directing a stream of cold water upon it. This has the effect of converting the sulfur into a plastic state rendering the treated body less brittle than it would otherwise be if allowed to cool slowly. The product is practically odorless and possesses desirable qualities of higher priced material.

Wood pulp, or other fibrous material, may be treated in the manner described and subsequently molded into suitable forms, to provide various articles of manufacture.

While I have herein described my process in minute detail, it will be manifest that changes in this specific manner of carrying the invention into effect may be made within the scope of the appended claim.

Having described the invention what I claim as new and desire to secure by Letters Patent is:—

The process of treating fibrous material to render it non-absorbent and to increase its insulating qualities and its texture, which consists in immersing it in a hot solution of sodium carbonate, to drive out resident content from the pores; then removing it from

the solution and drying it; then immersing it in a hot hydro-carbon liquid to neutralize the odor produced by the sulfur and to expand the pores; then drying it; then placing 5 it in a solution of sulfur and resin of commerce and maintaining it at temperature sufficient to keep the sulfur in a molten state

until the pores of the fibrous material are sufficiently filled, then removing the material from the vat and suddenly cooling it. 10

In testimony whereof I hereunto subscribe my name.

WILLIAM WEIMAR.